

Oct. 7, 1958

B. DOUGLAS

2,855,358

GALVANIC ANODE

Filed Feb. 1, 1955

4 Sheets-Sheet 1



Fig. 1



Fig. 2



Fig. 3



Fig. 4

INVENTOR.  
Burke Douglas

BY

Griswold & Burdick  
ATTORNEYS

Oct. 7, 1958

B. DOUGLAS

2,855,358

GALVANIC ANODE

Filed Feb. 1, 1955

4 Sheets-Sheet 2



Fig. 5



Fig. 6



Fig. 7



Fig. 8



Fig. 9  
INVENTOR.  
Burke Douglas

BY

Griswold & Burdick  
ATTORNEYS

Oct. 7, 1958

B. DOUGLAS

2,855,358

GALVANIC ANODE

Filed Feb. 1, 1955

4 Sheets-Sheet 3



Fig. 10



Fig. 13



Fig. 14

INVENTOR.  
Burke Douglas  
BY

Griswold & Surdick  
ATTORNEYS

Oct. 7, 1958

B. DOUGLAS

2,855,358

GALVANIC ANODE

Filed Feb. 1, 1955

4 Sheets-Sheet 4

Current Density Versus Distance from  
Anode Under Depolarized Conditions



Fig. 10

Percent of Total Current  
of Various Distances from Anode  
under Depolarized Conditions



Fig. 11

INVENTOR.  
Burke Douglas

BY

Griswold & Burdick  
ATTORNEYS

1

2,855,358

## GALVANIC ANODE

Burke Douglas, Freeland, Mich., assignor to The Dow Chemical Company, Midland, Mich., a corporation of Delaware

Application February 1, 1955, Serial No. 485,373

13 Claims. (Cl. 204—197)

This invention relates to the cathodic protection of metals and particularly to improved consumable anodes for use in cathodic protection systems.

Cathodic protection systems are well known in which a metal immersed in an electrolyte is protected from corrosion by means of a sacrificial or consumable anode which is immersed in the electrolyte and is electrically connected to the (cathodic) metal which is to be protected.

Sacrificial or consumable anodes comprise a metal which is anodic to the metal surface to be protected and some means, such as a metal core strap, rod or cable to attach the anode to the surface to be protected. When the anode and the surface to be protected, or cathodic surface, are in an electrolyte and are electrically connected together, the resulting flow of current between the two electrodes greatly reduces the rate of corrosion of the cathodic surface.

The cathodic protection of pipe lines, ship hulls, metal sea walls, and water tanks are examples of uses made of sacrificial anodes, such as magnesium anodes, for example. For many applications the expense of replacing anodes represents a substantial part of the cost of the protective system. Further, in the case of anodes attached to ship hulls, for example, the anodes may be replaced conveniently only at infrequent intervals, such as when the ship is in dry dock.

To avoid costly and frequent replacement of anodes, the use of large anodes which have a long useful life has become common. Large anodes, however, tend to provide larger currents than are needed for the protection of the cathodic surface and to that extent defeat their purpose of providing long-lived protection. Further, in marine service the larger anodes produce greater drag or resistance to the water passing the anodes than do smaller anodes and for this reason are undesirable for use on ships.

Resistance elements have been used in series with the electrical circuit between the anode and the cathodic surface to limit the current flow therebetween. Resistance elements give only a partial answer to the problem of extending anode life, however. Anodes are consumed as a result of chemical attack as well as by current flow, and the resistance element does not affect the rate of chemical attack. Thus, anode circuits including a resistance element operate at a lower efficiency (measured in ampere hours per pound of anode) than do anodes which are operated in systems not having series resistance elements included therein.

Anode efficiency, however, is but one criterion by which an anode is judged. Another indication of the worth of a galvanic anode is its throwing power or, stated differently, the cathodic area in which the anode provides adequate cathodic protection. The throwing power of anodes which are mounted close to the cathodic surface is quite limited since much of the current from the anode is used to protect areas of the cathodic sur-

2

face which are closely adjacent to the anode. Thus, the close-in areas are over-protected (by excessive current) and remote areas are inadequately protected. Resistor anodes, while limiting the total current, do not change the proportional distribution of the available current.

Another difficulty encountered in connection with galvanic anodes is that the anode consumption often follows a pattern such that the magnesium anode body (for example) becomes loosened from its mounting means or core while the body weight is still a significant percentage of the anode weight when installed. For cathodic protection purposes, the anodic metal is wasted which remains after the electrical contact between the core or anode mounting means and the anode body is broken or becomes a high resistance contact.

The labor cost for mounting anodes often represents a substantial part of the cost of the cathodic protection system, since men having several basic skills, such as welders, boiler makers, and painters may be used in mounting the anodes on a ship hull, for example. An anode which requires workers having only a single skill or trade to mount would therefore result in a saving in the cost of the cathodic protection system.

Difficulties due to uneven consumption of the anode in different parts thereof have likewise been encountered when one part of an anode is closer to a cathodic surface than is another part of the anode. A cathodically protected water heater in which the magnesium anode rod is inserted from either the top or the bottom of the tank is an example of an anode use in which the anode is subject to the above difficulty.

In such water heaters (or water softeners or similar tanks), the current flow to the supporting wall of the tank, which is very close to the attached end of the anode, is often excessive. The result is that the attached end of the anode may be entirely consumed long before the remainder of the anode is depleted. This irregular depletion of the anode is undesirable because it will result in anode inefficiency.

A principal object of this invention is to provide an improved galvanic anode which has a longer useful life per unit weight of anode material.

Another object of this invention is to provide an improved galvanic anode having improved current distribution to the cathode.

A further object of this invention is to provide an improved galvanic anode structure which needs no separate insulating means to separate the anode from the cathodic surface.

Yet another object of this invention is to provide an improved galvanic anode structure having means for selectively controlling the rate of anode consumption in various parts of the anode body.

In accordance with the invention, there is provided a galvanic anode comprising a consumable body portion and core means by which electrical connection between the anode and a cathode surface may be made, the anode being enclosed in an insulating covering or casing. When the anode is ready for use, the casing is provided with a plurality of apertures in at least one surface thereof.

The invention, as well as additional objects and advantages thereof, will best be understood when the following detailed description is read in connection with the accompanying drawings, in which:

Fig. 1 is a plan view of a plastic coated anode in accordance with the invention;

Fig. 2 is a side elevational view of the anode shown in Fig. 1;

Fig. 3 is a sectional view taken along the lines 3—3 of Fig. 1;

Fig. 4 is a fragmentary sectional view, on an enlarged scale, showing the plastic coating extending over the mounting strap;

Fig. 5 is a sectional view taken along the lines 3—3 of Fig. 1 and showing the anode consumption pattern after partial consumption of the anode shown in Fig. 1;

Fig. 6 illustrates an anode of the type shown in Fig. 1 as mounted on the side of a ship hull;

Fig. 7 is an elevational view of a plastic coated anode in accordance with the invention which is especially adapted for use with small metal-hulled craft and which requires no underwater connection to the hull of the craft;

Fig. 8 illustrates an anode in accordance with this invention which is adapted for use in water heaters or like uses;

Fig. 9 illustrates a cable-cored coated anode in accordance with the invention;

Fig. 10 is a graph showing output current as a function of exposed anode area;

Fig. 11 is a graph showing the percent of total anode current at various distances from the anode under initial operating conditions;

Fig. 12 is a graph showing current density versus distance from anode for three types of anodes under initial operating conditions;

Fig. 13 is a graph showing the current distribution (under initial conditions) of a perforated anode in accordance with this invention and a bare anode restricted with a resistor when the total current outputs of each anode are equal, and

Fig. 14 is a graph showing current density versus distance from the anode for a bare anode and a coated and perforated anode under conditions of continued operation (i. e., after 24—30 hours of operation).

Referring to Figs. 1 through 4 there is shown a galvanic anode indicated generally by the numeral 20 and comprising a consumable body 22, made of magnesium, for example, and having a metal core 24 (such as steel) embedded in the magnesium and bonded thereto and extending therefrom as a mounting strap 24a. The anode is encased in a plastic cover 26 which fits closely about the anode body 22 and mounting straps 24a. The top of the plastic cover 26 contains a plurality of apertures 28 which are illustrated as being round although apertures of other configurations may be used. It should be noted that no apertures 28 appear in that part of the plastic coating which lies directly above the cores 24.

Referring particularly to Fig. 4, the plastic cover 26 extends along at least a part of the mounting straps 24a. The mounting straps 24a usually contain a plurality of bores 30 which serve two purposes. The bores 30 in the straps provide a convenient means by which the anode 20 may be bolted to a supporting structure. Also, the plastic cover 26 which extends on each side of the straps 24a flows through at least one of the bores 30, causing the plastic on opposite sides of the strap to be bonded to itself. Such bonding of the cover 26 lessens the likelihood that the plastic cover 24 will tear off the mounting straps 24a and thence tear off the anode body 22. In practice, the plastic cover 26 may entirely cover the mounting straps 24a, but may be cut back to the desired point when the anode 20 is to be mounted.

The plastic cover 26 is a dispersion resin coating of dispersion grade polyvinyl chloride resin or vinyl chloride copolymer resins plus plasticizer and stabilizer. Such anode coatings are electrically insulating and are physically tough. A coating thickness of  $\frac{1}{8}$  inch has been found to be sufficient for most applications.

A specific coating formulation which may be used comprises:

60 parts by weight of polyvinyl chloride plastisol

40 parts by weight of di-octyl phthalate

1 part by weight of stabilizer such as "Thermolite 31"

which is an organo-tin chemical sold by the Metal and Thermit Co. of New York, N. Y.

5 parts by weight of mineral spirits such as Apco thinner

The plasticizer used is one which is relatively ineffective at room temperatures. However, when an anode which is heated to 350° to 400° F., for example, is dipped into the dispersion, the heat increases the activity of the plasticizer and a resinous coating is formed on the hot surface of the anode.

10 While the coating of the general type described above proves very satisfactory, other coatings may be used. For example a coating may be applied by hot dipping an anode into an ethyl cellulose gel lacquer. Alternatively, the anode may be coated with neoprene which has an advantage in that such a coating would be relatively immune to attack by light hydrocarbons. Specifically neoprene coated galvanic anodes are well adapted for use in cathodically protecting gasoline tanks or compartments in tank ships.

15 As cast, dip coated anodes in accordance with this invention often contain a groove 31 in their top surface 32 which is disposed about  $\frac{1}{4}$ " from the peripheral edge of the anode body. The groove 31 is about  $\frac{1}{8}$ " wide and about  $\frac{1}{8}$ " deep. When the coating or cover 26 is applied by dipping (or spraying, painting, etc.) the groove 31 becomes filled with a rib 33 of the coating material. During use, the rib 33 of coating which extends into the groove 31 lengthens the ion path through 20 the electrolyte to the upper edge of the anode body 22. As the anode body 22 is consumed, the peripheral surface portion of the body tends to remain as a shell to keep the plastic cover 26 tightly in place over the anode body 22. The result is a neater anode which has more resistance to tearing of the cover 26 from the anode body 22 than does a partly consumed anode in which the sides of the anode body 22 are consumed and the cover becomes loose.

25 One of the advantages of anodes made in accordance with this invention is illustrated in Fig. 5. As the plastic covered anode 20 is consumed during use, the surface 32 of the anode which lies below the apertures is primarily consumed, leaving relatively untouched the anode surface under that part of the cover 26 where there are no apertures 28. While the entire upper surface of the anode body 22 will eventually be consumed, the surface area under the apertures 28 in the cover 26 will be "eaten away" the fastest. The result is that the magnesium anode body 22 will remain firmly bonded to the cores 24 even though the distance between the surface 32 and the bottom 34 of the anode on either side of the cores 24 is less than the space between the core 24 and the bottom surface 34 of the anode. In an anode 20 of the above type, almost the entire body weight of the anode gives 30 useful cathodic protection.

35 Fig. 6 illustrates an anode 20 of the type shown in Fig. 1 as attached to a ship's hull 36. The anode is attached by welding the ends of the mounting straps as at 38 to the hull. Because anodes made in accordance with this invention require no additional insulation device or electrical control to separate them electrically from the cathodic surface, the cost of the anode installation, particularly the labor cost, is materially reduced as compared with the cost of installing a bare anode.

40 The theory concerning the operation of the anodes of this invention is not fully understood. As has been observed, for an electrolyte of given electrical conductivity and assuming a cathodic surface to be protected which is large with respect to the anode, the current output of the anode 20 may be controlled by regulating the number and size of the apertures, thus controlling the flow of current from the surface of the anode 20. The top surface of the anode is conveniently used for this purpose. It is also known that the current output of various parts 45 of the anode surface may be controlled by the size and

number of apertures 28 above the various parts of the anode surface.

Data is given concerning operation of anodes of this invention under both depolarized and polarized conditions. As the term is used herein, depolarized conditions are those in which the anode and cathode are each at their natural potential while uncoupled in sea water. Under polarized conditions, as the term is used herein, the anode is at its natural potential while the cathode is at a potential which is a function of both the current density and the length of time the current from the anode has been flowing to the cathode. In the tests made for the purpose of gathering data for the graph in Fig. 14, it was found that after 24-30 hours the potentials tended to remain constant as if a steady state condition of operation had been reached.

The graph shown in Fig. 10 shows the relationship between the anode current (in milliamperes) and the "exposed anode surface area" (measured in square inches of opening in the cover 26) for different types of anodes. The term "exposed anode surface area" as used herein refers to the area of the apertures in the coating. It is realized that in partly consumed anodes, however, the surface area exposed to electrolyte may be larger than the aperture area. The ion path to the cathode remains the same (i. e., through the apertures). The coated anode data for the graph in Fig. 10 were obtained by varying the number of  $\frac{5}{8}$ " diameter apertures 28 in the top surface 32 of a coated anode. However, the current line 40 in Fig. 10 is approximately the same when apertures 28 of other diameters (but of the same total area) are used.

As a practical matter, the aperture diameter is chosen depending upon at least two factors. First, the strength of the covering 26 of the anode should be maintained at a high value in order to lessen the tendency of the cover 26 to tear away from the anode body 22 when subjected to external forces. Secondly, the apertures 28 must be large enough to permit the anode corrosion product to be washed out of the casing. The anode material may influence the characteristics of the corrosion product.

For anodes used in moving water, cover apertures 28 which are  $\frac{5}{8}$ " in diameter have proven very satisfactory. The thickness of the cover 26 may vary according to the material used and the installation of the anode, that is, whether the anode will be used in quiet or fast moving electrolyte. In anodes coated with a polyvinyl chloride type coating a thickness of .09" proved satisfactory for use in water moving at a speed of 25' per second.

In tests of bare anodes and coated anodes placed in sea water under the same operating conditions, it has been found that substantially no calcareous coating builds up on the cathodic surface around a coated anode mounted against a steel bulkhead in sea water while a substantial calcareous coating is built up around an uncoated or bare anode.

While the existence of a calcareous coating is evidence of excessive current, it is also evidence of paint damage and unsightliness. To the owner of small sea-going craft, the physical appearance of such craft is of prime importance. Anode currents strong enough to cause calcareous deposits cause the deterioration of the paint on that portion of the hull which is in the high current density area. The results have been that most ship owners have heretofore been reluctant to solve their hull corrosion problems at the expense of having an unsightly hull or damaged paint.

As is clearly seen from Figs. 11, 12 and 14 the current density on the cathode close to the coated anodes is only a small fraction of the current density on the cathode close to the bare anode under both polarized and depolarized conditions of operation. As shown in Figs. 11 and 13, the use of a perforated coated anode results a substantial saving in "close-in" current over a resistor restricted bare anode of equal current output.

Fig. 11 shows the percent of total current versus distance from the anode under depolarized conditions. It may be seen from this graph that although coating the sides of the anode results in a considerable saving in current at distances close to the anode, the coated and perforated anode of this invention results in a further and substantial reduction of the current to cathodic surfaces which are close to the anode. Bare anodes are even more wasteful of their current output.

The anode test setup used in securing the data for the graphs of Figs. 11-14 comprised a series of concentric annular cathode segments made of steel with the test anode mounted in the center of the annular cathode segments. The cathode segments were insulated from each other and each had a flat top surface approximately 3" wide (as measured radially from the center of the annulus). The test setup included 8 of such cathode segments, mounted concentrically as stated above. When the graphs of Figs. 11-14 inclusive are read, it should be remembered that the current density readings are actually for areas rather than for points as might be assumed from the distance scales on the graphs.

In the gathering of the data for Figs. 11-14, a steel cathode was used and all the anodes used in the tests were identical in size and shape. The anodes were cylindrical in shape, having a diameter of 3" and a height of 4", and were made of cell grade magnesium. One anode was bare, one anode had its side coated and top bare, and one anode was entirely coated and contained all the  $\frac{5}{8}$ " diameter perforations which could conveniently be made in the top surface thereof with  $\frac{5}{16}$ " spacing between adjacent apertures. The bottom surface of each of the anodes was coated to protect that surface from the cathodic surface to which the anode was mounted. The measurements were made with the anodes immersed in sea water moving at a rate of approximately 6 ft./minute. In those graphs where current values are given, no attempt should be made to relate the currents to that current which is necessary to protect the cathodic surface. The experimental data shows only current distribution from the anode without regard to the current required to achieve protection. Obviously, if more current is needed, larger anodes may be used.

Fig. 12 shows current density versus distance from anode under depolarized conditions of operation. The graphs of Figs. 11 and 12 were plotted using the same experimental data. It should be noted in Fig. 12 that the current density close to the anode (3" from the anode) is about 7 times as high for a bare anode as for a perforated and coated anode in which the perforations were placed as described above. Also, a perforated and coated anode puts a larger part of its output current farther away from the anode than does the bare anode. This larger far-out current tends to increase the cathode area protected by a coated anode as compared with bare anodes of similar current capabilities. It should be realized that in the graphs of Figs. 11 and 12 the total output current of each of the anodes is different from the output current of the others.

The graph shown in Fig. 13, however, shows current distribution under depolarized conditions in the case of equal total currents of a bare anode whose current output is restricted by a series resistor and a perforated coated anode. It should be noted that the "close-in" current of the perforated coated anode, that is, the current going to the cathodic surface which is closely adjacent to the anode, is considerably lower than the close in current of the resistor-restricted anode. This graph indicates that the resistor in the resistor-restricted anode apparently restricts only the total current output of the anode and has little effect on the current distribution pattern of the anode. Compared with Fig. 11, the percent of current output curve for the bare anode is very similar to the corresponding curve for the resistor-restricted anode. Referring again to Fig. 13, it may

be seen that in the case of the coated and perforated anode only about 8% of the total current was used within 3 inches of the anode whereas about 23% of the total current of the resistor-restricted anode is utilized in the same area within 3 inches of the anode.

Considering the current distribution curve of Fig. 13, it appears to now be feasible to install anodes on surfaces which remain depolarized and still achieve long lived protection. Previously on such continually depolarized surfaces, such as on a ship's rudder, the anodes were quickly depleted due to the excessive close-in current. Anode life of bare anodes in such installations was much less than the anode life of bare anodes when installed adjacent to polarized surfaces. Since ship anodes may be installed conveniently only when the ship is in dry dock, the result has been that ship hulls have not been protected as uniformly as desired because of inability to replace anodes which were rapidly depleted. The coated and perforated anode provides an answer to this problem by providing a controlled distribution of current and thereby making possible more uniform protection of a ship's hull or other cathodic surface.

A comparison is shown in Fig. 14 between a coated and perforated anode and a bare anode of equal size regarding current density versus distance under polarized conditions of operation. Fig. 14 shows that the close-in current of the bare anode at 3" distance from the anode is about 4 times the close-in current of a coated and perforated anode. Thus, even under polarized conditions of operation, the bare anode is quite wasteful in the usage of its current output in providing close-in protection to a cathodic surface.

It should further be remembered that under conditions where the cathodic surface is in rapidly moving electrolyte, as for example on the hull of a ship, the hull seldom becomes completely polarized.

Another practical advantage accrues to the use of coated and perforated anodes which is not apparent from the graphs. Often the cathodic surface to be protected is coated, as by painting, and the coating effectively reduces the area of the exposed cathodic surface so far as anode current requirements are concerned. However, when high close-in currents occur, the coating peels off and an enlarged, bare cathodic surface is presented to the anode. The bare surface in return requires more total current from the anode in order that the bare surface be adequately protected. Because of the substantial reduction in close-in current when anodes of this invention are used, the paint or coating on the cathodic surface is relatively unaffected. It should be realized, however, that a very few brands of paint that were tested peeled off with even very low current to the cathodic surface.

To cite an example of the different current requirements for equal area surfaces, a galvanized water tank may, and often does, require 10 times the anode current for effective protection as does a glass lined water tank of equal size. A painted surface would not be as good as a glass lined surface in reducing the current required for protection. However, it can be appreciated that any loss of paint from the cathodic surface would increase the anode current demand and, if effective protection is to be maintained, would shorten the effective life of the anode. Thus, the fact that paint is not removed from the cathodic surface when coated and perforated anodes are installed results in further important advantage in extending the life of the anode.

The galvanic anode structures thus far described have been of the type which are bolted, welded, or otherwise fixedly attached to a structure which is to be cathodically protected. Referring to Fig. 7, there is shown a plastic coated galvanic anode 42 of generally cylindrical form. A metal mounting strap or cable 44 extends from the anode body and is bonded therein. The plastic coating

or covering 46 of the anode is provided with perforations 48 (apertures) in order to regulate the current flow from the anode as previously described in connection with other coated and perforated anodes. The plastic coating 46, as illustrated, usually extends at least part way along the mounting strap or cable 44. The plastic coating or covering of the anode 42 also provides an anode which is cleaner to handle than is a bare anode. It is anticipated that anodes of the type shown in Fig. 7 will find use as readily demountable anodes for use on small vessels. In this type of application, the anodes would normally be stowed away except when the vessel was anchored or tied up at a dock or pier. The anode strap would then be fastened to a cleat mounted on the metal hull of the vessel, completing the protective electrical circuit. Such an anode arrangement has merit for small craft use, since many pleasure craft are docked or anchored far more hours than they are operated. The demountable anode provides cathodic protection, yet may be removed easily so there is no extra "drag" in the water. The plastic covered anode is neater and more desirable, from a housekeeping standpoint, than is a bare anode. Further, since galvanic anode surfaces become roughened during their consumption and often have small, sharp edges, the plastic coating over the anode results in an anode assembly which is safer to handle than a bare anode. The anode structure may be included as part of or combined with the fenders of the vessel if desired, thus eliminating a separate object to be stowed while the vessel is in use. The covering 46 of the anode 42 need not be applied by dipping the anode body in liquid plastic, but may comprise a permanent casing in which bare anodes may be disposed. Anodes and casings of this general type are described and claimed in applicant's copending application, Serial No. 485,438, filed February 1, 1955.

While the advantages of the coated and perforated anodes of this invention have been described mainly in connection with ship hulls, such anodes have many other applications.

For example, coated anodes having no perforations may be stock piled and stored without shelter from the weather for long periods of time without loss of anode weight by corrosion. Such anodes are provided with perforations of the required number and size at the time they are sold (or are to be used) for the particular installation in which they will be utilized.

Different corrosion prevention applications require anodes of many different varieties of performance characteristics. To stock all types of anodes would place a considerable financial burden on a distributor or dealer. However, when a distributor stocks coated but unperforated anodes in accordance with this invention, a minimum number of anode types and sizes serves to supply the anodes for a wide variety of application situations when the anodes are given the required perforation pattern.

The availability of an unperforated coated anode is also attractive to corrosion engineers who prefer to maintain some degree of secrecy about their ideas as to what is the best solution to a particular corrosion problem.

Coated and perforated anodes may be used in many applications where resistor-restricted anodes or bare anodes are now used. Pipe line cathodic protection systems can make use of the anodes of this invention by mounting the anodes closer to the line than heretofore has been practical because of the excessive local current to the nearby pipe.

The use of a coated and perforated anode in a water tank is illustrated in Fig. 8. The anode, indicated generally by the numeral 50, extends upwardly from the bottom of the tank 52, but could be mounted to extend downward from the top of the tank. In either method of mounting, excessive current usually flows to the mount-

ing end of the tank because the surface 54 from which the anode 50 is mounted is closer to the mounting end of the anode 50 than are the sides of the tank 52. Thus, the lower end of the coating 56 on the anode 50 in the tank has smaller apertures 58 than appear in the coating over the remainder of the anode. The smaller apertures 58 near the bottom end of the anode restrict the current which flows from that part of the anode, thus causing a more uniform expenditure of the anode than would occur if the anode apertures were all uniform in size. Such selective current flow from the anode 50 would not be possible in a resistor-restricted anode. In addition, the coating 56 provides physical support for the anode 50.

Fig. 9 illustrates a cable-core coated and perforated anode, indicated generally by the numeral 60, made in accordance with this invention. The anode coating 62 extends along the mounting cable 64 for a considerable distance from the anode body 66 to prevent strong local current flow between the anode and the nearby mounting cable 64. Such cable anodes are well adapted to be clamped to a submersible metallic net, for example. The size and number of perforations 68 of the anode may be varied to accommodate a wide variety of corrosion control situations.

Any of the anode assemblies described above may be coated with an anti-fouling coating in addition to or as a substitute for the previously described coatings. An anti-fouling coating which is suitable for use on anodes for use in sea water is a copper salt of polyacrylic acid. Such coatings can be made relatively insoluble by controlling the degree of polymerization of the coating material. The coating is physically tough and has a double anti-fouling action. The copper is toxic to small marine organisms and since the surface of the coating dissolves at a slow rate, the organisms cannot readily adhere to the coating.

As a precaution against baring the anode due to the dissolving of the anti-fouling coating, or because of the electrical properties of some coatings it is sometimes advisable to provide an under coating of normally insoluble material (such as described previously herein, for example), prior to applying the anti-fouling coating.

Another anti-fouling coating may be provided by dispersing copper particles through the non-soluble coating materials.

Another use of slowly soluble coating materials is to provide a delayed action anode for use in installations where mounting the anodes is expensive or can be done only at infrequent intervals. Thus, an immediately operative anode and a "delayed action" anode may be installed together with a coating on the delayed action anode which is calculated to expose the galvanic metal of that anode at approximately the time of the end of the useful life of the immediately operative anode.

It is now customary to attempt to achieve long-lived cathodic protection by the use of larger and larger anodes. Large anodes, while providing protection over a longer period than do smaller anodes, have higher current flow and thus are inefficient. Two small anodes, one of them a delayed-action anode, may be used to provide continuous protection without the inefficiency of a single large anode.

Among the suitable coatings which will slowly dissolve are polyacrylic acid (or salts thereof), polyvinyl alcohol, methyl cellulose plus enzyme, or natural gums plus bacteria. Arayakraya is an example of a natural gum which may be used. It is realized that not all the above coating materials are suitable for use in mobile installations such as ships. However, many stationary or seldom moved metals in sea-water or other saline electrolyte may be given long range protection by such delayed action anodes.

Delayed action anodes may likewise be used in tanks which are used to store or transport petroleum products

or other materials. The anode coating for such delayed action use is chosen from substances which have low solubility rates in the electrolyte to which they will be exposed.

Thus, it is apparent that the present invention provides improved galvanic anodes which have longer life, have better current distribution, are easier to store, and are more adaptable to a wide variety of corrosion control situations than are conventional bare anodes or resistor-restricted anodes.

I claim:

1. A rectangular block-shaped galvanic anode assembly comprising a magnesium anode body, a metal core embedded in said anode body and bonded thereto, said core extending from said anode body, and a closely fitted coating of electrically insulating liquid impervious material surrounding said anode body, said coating containing perforations adjacent to at least one surface of said anode body, said perforations are each equivalent to or exceed in area the area of a circle having a diameter of one-eighth inch.

2. An assembly in accordance with claim 1, wherein said perforations are of varying sizes in different areas of said coating.

3. A galvanic anode assembly comprising a block-like anode body of a galvanic metal, a strap-like core embedded in and bonded to said body and extending therefrom as mounting means for said assembly, and a closely fitting coating of electrically insulating liquid impervious material surrounding said anode body and extending onto said mounting means, said coating containing perforations on a part thereof which faces at least one surface of said anode, said perforations are each equivalent to or exceed in area the area of a circle having a diameter of one-eighth inch.

4. A galvanic anode assembly comprising a generally rectangular block-like anode body of galvanic metal, said anode containing a depression adjacent to and extending along the peripheral edges of a major surface thereof, a metal core embedded in and bonded to said body, said core extending from said body as the mounting means for, and a closely fitting insulating coating surrounding said anode body and extending into said depression, and a plurality of apertures in that part of said coating lying above the anode area bordered by said depression.

5. A galvanic anode assembly comprising a generally rectangular block of galvanic metal, at least one metal strap-like member extending through said block and bonded thereto, said member extending from said block on each side thereof, said block being covered by a closely fitting coating of flexible, electrically insulating, liquid impervious material, an array of apertures in that part of the coating which covers at least one surface of said block, the apertures being so disposed that the area of the coating lying above said strap-like member contains no apertures.

6. A galvanic anode assembly comprising a generally rectangular block of galvanic metal, at least one metal strap-like member extending through said block and bonded thereto, said member extending from said block on each side thereof, said block being covered by a closely fitting coating of flexible, electrically insulating, liquid impervious material, the coating extending onto that part of said strap-like member which extends from said block, an array of apertures in that part of the coating which covers at least one surface of said block, the apertures being so disposed that the area of the coating lying above said strap-like member contains no apertures.

7. An assembly in accordance with claim 6, wherein said coating is a vinyl dispersion coating.

8. An assembly in accordance with claim 6, wherein said coating is a copper salt of polyacrylic acid.

9. An assembly in accordance with claim 6, wherein

**11**

said apertures are each equivalent to or exceed in area the area of a circle having a diameter of one-eighth inch.

10. An assembly in accordance with claim 6, wherein said apertures are of circular configuration and are five-eighth inch in diameter.

11. An assembly in accordance with claim 6, wherein said coating is at least .09 inch thick.

12. An assembly in accordance with claim 6, wherein that part of said member which extends from each side of said block contains an aperture through each extension and said coating on each side of said extension is bonded to itself through said aperture.

13. A galvanic anode assembly comprising a block-body of galvanic material, a metal core disposed in and bonded to said galvanic material, a close fitting coating 15 of electrically insulating, liquid impervious material surrounding said anode, said coating containing an array of apertures, said array covering a substantial area of

5 at least one surface of said body, said apertures each being equivalent to or exceeding in area the area of a circle having a diameter of one-eighth inch, and means for mounting said anode, said means being in electrically conductive contact with said metal core.

**References Cited** in the file of this patent

**UNITED STATES PATENTS**

915,846 Friedheim ----- Mar. 23, 1909

**FOREIGN PATENTS**

504,585 Belgium ----- July 31, 1951  
1,081,845 France ----- May 6, 1953

**OTHER REFERENCES**

Marine Eng., vol. 58, No. 6, June 1953, pp. 69-73.